

No. 870,620.

PATENTED NOV. 12, 1907.

H. FRASCH.  
MINING SULFUR.  
APPLICATION FILED OCT. 30, 1903.



J. H. Schott } Witnesses  
J. J. Burch

No. 870,620.

PATENTED NOV. 12, 1907.

H. FRASCH.  
MINING SULFUR.

APPLICATION FILED OCT. 30, 1903.

2 SHEETS—SHEET 2.



# UNITED STATES PATENT OFFICE.

HERMAN FRASCH, OF NEW YORK, N. Y., ASSIGNOR TO THE FRASCH SULPHUR PROCESS COMPANY, OF KITTERY, MAINE, A CORPORATION OF MAINE.

## MINING SULFUR.

No. 870,620.

Specification of Letters Patent.

Patented Nov. 12, 1907.

Application filed October 30, 1903. Serial No. 179,232.

To all whom it may concern:

Be it known that I, HERMAN FRASCH, a citizen of the United States, residing in the city of New York, borough of Manhattan, and county of New York, in the 5 State of New York, have invented new and useful Improvements in Mining Sulfur, of which the following is a specification.

This invention relates more particularly to the obtainment of sulfur from an underground deposit by 10 melting the sulfur therein and removing it therefrom in the melted condition; but each of the improvements constituting the invention is intended to be secured for all the uses to which the same, with or without modification, may be adapted.

15 Heretofore I obtained a patent, No. 461,429, dated October 20, 1891, for the process of obtaining sulfur in the aforesaid manner, and a patent, No. 461,430, also dated October 20, 1891, for apparatus to be used in so obtaining the same. In accordance with what was 20 then considered the best mode of working, water heated to a temperature above the melting point of sulfur was introduced through suitable piping into the underground deposit and afterwards returned by other piping to the surface of the ground at a temperature somewhat 25 lower, but still above the melting point of sulfur. The sulfur, melted in the underground deposit, was raised to the surface through a proper pipe by the pressure produced in the deposit by pumping the hot water thereinto (the return water being held under sufficient pressure) or by the direct lifting action of a pump placed 30 in the deposit. Subsequently, to wit, on May 27, 1897, I filed an application (officially numbered 638,357) for a patent on certain improvements, which were more particularly designed for the obtainment of sulfur as 35 aforesaid from deposits in porous rock, flooded with natural water, such as had been encountered in actual working. Without here attempting a full recital, it may be observed that said application discloses, among other things (1) the melting of the sulfur in a porous

40 water flooded deposit by means of water heated above the melting point of sulfur and, indeed, most advantageously above the temperature at which melted sulfur begins to darken, and introduced into the deposit without return, being forced out through the porous 45 rock and flowing away underground, and (2) the raising of the melted sulfur to the surface of the ground by the aid of compressed air introduced into the column of melted sulfur in sufficient volume to render the average density of said column low enough for its pressure to be 50 overbalanced by the otherwise inadequate pressure attainable in the porous deposit. The raising of the melted sulfur as set forth in my said application has been found satisfactory; and the present invention does not concern itself with that part of the general 55 process. The melting of the sulfur as set forth in said

application, while correct in principle, has been found to admit of some further improvements; and to it the present invention relates. By melting as described in said application, the expense per ton of sulfur obtained is decreased and the average yield of sulfur per well increased beyond anything believed to be possible in the case of a water flooded porous deposit with a circulation (that is, with introduction and return) of hot water; but, nevertheless, such melting has not, for all wells, given the expected results. In several instances 60 wells had to be abandoned at a loss; because there was no recovery from them of sulfur sufficient to compensate for the expense connected with the installation and working. I have discovered that the difficulty was mainly due to the water naturally present in the 65 rock, whose existence I knew about and the effects of which I partly appreciated and had largely succeeded in counteracting by proceeding as set forth in my said application; although the difficulty seems (as I have also discovered) to be due in part to the existence in or 70 above the deposit of passages so large as to allow much hot water to flow away without proper effect.

75 In accordance with the present invention, comminuted material (sawdust is considered the best and is more especially claimed, although my claim extends 80 also to suitable comminuted material in general) is introduced into the deposit so as to fill the larger passages in the rock and thus effect the distribution of the hot water more uniformly in the neighborhood of the pipe up which the sulfur is raised. Further in accordance 85 with the present invention the rate at which the hot water is sent into the underground deposit and caused to flow away through the rock is increased sufficiently beyond the rate mentioned in my said application to prevent the inroads into the melting space of the naturally 90 present water from the surrounding rock. In my said application, by way of example and as illustrating what was then considered the best mode of working, three heaters for the fusion water are shown and one hundred and twenty five gallons of water per minute is mentioned as cold water supply for a single heater. To this would be added the water from condensing steam necessary to raise the cold water to the steam's temperature, say, a total for the three heaters shown of about 500 gallons (about two tons in weight) 95 of hot water introduced each minute into the mine (or underground deposit) and caused to flow away through the rock. In accordance with the present invention, this rate of about 500 gallons (or two tons) per minute is materially increased. The rate of about 1,250 gallons (say, about five tons) per minute has been found to give satisfactory results; but there is reason to believe that a further increase would give at least as good results; and it is not intended to restrict the claim on 100 this feature of the present invention to a delivery of 105 110

1,250 gallons (5 tons) per minute as either a minimum or a maximum.

In order to increase the rate of delivery of hot water into the deposit without increasing the size of the mine piping, it is found expedient to supply such water to the mine piping at a pressure above that which corresponds with its temperature when it leaves the heaters; that is to say, in case the fusion water is raised by condensation of steam therein to the temperature of said steam, the so heated water is supplied to the mine piping under a pressure greater than that of said steam. This additional pressure can best be applied to the water between the heaters and the mine piping. It is applied when the underground porous deposit does not admit a pressure therein equal even to the pressure corresponding with the temperature of the hot water, when added to the pressure of a water column the length of the mine piping.

Other parts, improvements or combinations are included in the invention as hereinafter set forth.

The invention includes the apparatus herein set forth, its parts, improvements and combinations as specified.

In the accompanying drawings, which form part of this specification: Figures 1 and 2 are diagrams of a sulfur-mining plant, Fig. 1 being partly in vertical section and partly in elevation and Fig. 2 in plan. Fig. 1<sup>a</sup> is a detail view, showing a valve on the sulfur pipe, and Fig. 1<sup>b</sup> a detail view, showing a part of a water heater.

The feathered arrows show the flow of steam or air, the unfeathered arrows without cross-bar the flow of water, and the unfeathered arrows with cross-bar the flow of melted sulfur, the same being mingled with air.

So far as concerns the well itself, a single line of mine piping could be used alternately to introduce the hot water, without return, into the underground deposit and to convey the melted sulfur to the surface of the ground; but it is better to use at least two lines of piping, one for conveying the hot water and the other for raising the melted sulfur, and, when not so employed and it is so desired, for conveying hot water to the deposit; and it is still better to use two lines of hot water piping in addition to the sulfur pipe.

The pipe A is sunk through the ground to the rock; and a hole in continuation of the pipe bore is drilled into or through the sulfur-bearing deposit C, the rock B immediately below the pipe A being strengthened (when considered necessary or expedient) by cement.

In an application of February 6, 1905, which is officially numbered 244,508, and is in part a continuation of my hereinabove mentioned application of May 27, 1897, I have more fully described such strengthening of the rock; and I have also specified the same in claims which I have made in said application 244,508.

When the well hole is ready, the inner hot water pipe D, the sulfur pipe E and a pipe F for discharging compressed air into the lower part of the column of melted sulfur are inserted. The hot water pipe D (as shown) has a plug D', with a perforation therein through which the sulfur pipe E passes. On said plug D' the collar E' of said pipe E rests. The lower end of the pipe E (as shown) opens into a strainer D'' formed by an extension of the pipe D. The wall of the pipe D just above the plug D' is perforated for the escape of

hot water into the mine. The wall of the strainer D'' is perforated so as to let in the melted sulfur, but to keep out solid particles.

The piping is best made of iron or steel with a protecting layer of a metal, such as zinc or aluminium, which is not corroded by sulfur, over those portions of the piping liable to be in contact with the melted sulfur.

As so far described, the well is the same as shown in my said application 638,357. It could, of course, be otherwise constructed, so far as the present invention is concerned; since this latter contemplates any proper piping for conveying the hot water into the mine without return and for removing the melted sulfur therefrom. A feature of the present invention consists, however, in introducing hot water which flows away underground partly through the sulfur pipe and partly through a separate hot water piping, the introduction of hot water through the sulfur pipe being, of course, at a time when the same is not in use for raising sulfur.

A valved branch e is shown for supplying hot water, when desired, to the sulfur pipe. The branch e' serves to convey the melted sulfur and is closed by a stop-cock e'' (Fig. 1<sup>a</sup>), when the sulfur pipe is used for introducing hot water into the deposit. The stop-cock on the branch e' may be of any suitable description. Its construction is no part of the present invention. I have, however, devised a valve which is specially adapted for pipes which convey melted sulfur, the same forming the subject of my application No. 179,231, filed of even date herewith; and Fig. 1<sup>a</sup> exhibits such valve in elevation.

At d and a are valved branches for supplying hot water to the mine pipes D and A, respectively. The pipe A may advantageously be ten inches in interior diameter, the pipe D six inches, the pipe E three inches, and the pipe F one inch. The length of the pipes will, of course, depend upon the depth of the sulfur deposit below the surface of the ground.

So far as concerns the heating of the water to above the melting point of sulfur, any suitable heaters may be used; but it is considered advantageous and a special improvement to employ those in which live steam of appropriate temperature is condensed in the water to be heated. Six heaters G of this description are shown. Each of them receives the live steam from the steam main K through a valved branch 2 and the water to be heated from the cold water main L through a valved branch 3. The water is, of course, delivered under sufficient pressure to force itself into the heater against the pressure of the live steam therein. This may be advantageously 90 pounds to the square inch above atmospheric pressure, or even more, if steam of the higher pressure and temperature be found not to make the fusion water so hot that it would render the sulfur in the pipe E pasty and thereby interfere with its flow. Steam of between 95 and 100 pounds' pressure has been successfully used. Each heater G has appliances inside for bringing the water and steam into intimate contact with each other, so that the water attains the steam's temperature. Preferably the appliances of my said application of May 27, 1897, No. 638,357, would be used. They consist (see Fig. 1<sup>b</sup>) of a stack of pans g (a few of which only are shown) set one upon another and held apart by the legs, by

which they are supported. In the bottom of each pan are perforations surrounded by low rims, so that each pan will contain a layer of water with a steam space between it and the under side of the pan above. In consequence of official requirement of division holding the water heating means to be a separate invention from the other matters of said application of May 27, 1897, said means have been made the subject of a divisional application which was filed February 6, 1905, and has been officially numbered 244,510.

Each heater discharges the hot water through a valved branch pipe 4 into the first hot water main M. From this main the pumps N are supplied, each through a valved branch 5. As shown, n is the pump cylinder, n' the steam cylinder, and n'' the rod between the pistons of a pump. The pumps N deliver the hot water each through a valved branch 6 into the second hot water main P, which supplies it through the branches d and a to the hot water mine piping D and A and also 20 through the branch e to the sulfur pipe E, when this is not being used for elevation of sulfur and it is desired to send hot water down it into the deposit.

By the operation of the pumps N, the water which left the heaters G at the temperature corresponding 25 with its pressure, namely, at the temperature of the live steam in the heaters G, to the pressure of which steam it was subjected, is supplied to the mine piping at a higher pressure. Thus more hot water is delivered through given mine piping than would be the case 30 if such water was delivered to said piping at the pressure corresponding with its temperature on leaving the heaters G.

With pipes A and D of ten-inch and six-inch bores, respectively, the rate at which the hot water is sent 35 into the underground deposit by the pumps N through said pipes and caused to flow away underground can be increased sufficiently beyond the rate mentioned in my said application to prevent inroads from the surrounding rock of the water naturally present therein 40 and thereby to increase materially the amount of sulfur which can be obtained from a well having hot water pipes of the respective bores named.

The hot water may be sent by the pumps N into the deposit C at the rate of about 1,250 gallons (about five tons in weight) per minute; and its introduction at this 45 rate has resulted in obtaining a much larger average yield of sulfur from wells than was obtained when the hot water was introduced at the lesser rate mentioned in my said application. The difference is evidently not due merely to the amount of hot water introduced; for in such case the wells would in the end yield on the average as much sulfur with the slower as with the more rapid introduction of the hot water. A time element is involved, the effect of which could 55 not be, as in fact it was not, anticipated.

Should it appear that the sulfur is not melting properly (as shown, for example, by the slackening of the yield of melted sulfur), or that the hot water is not sufficiently distributed in the neighborhood of the well 60 (as shown by the too free working of the pumps N and the appearance of the water glasses attached to the heaters G) and especially if, as is most apt to be the case, the process appears to be working improperly in both these respects, sawdust is pumped into the mine 65 piping.

For this purpose a mixing tank Q is shown, having a stirrer q, a water supply 7, and a discharge pipe 8 leading to the inlet of one of the pumps N. The stirrer q is less important than the other parts, as the stirring can easily be effected by a shovel or other instrument 70 in the hands of a workman.

The tank Q may be open at the top; and the water supply 7 may deliver water at about 212° F.; but it is not essential that the tank be open; nor is any particular temperature essential for the water which is introduced into the tank Q for mixing with the sawdust.

The mixture of sawdust and water from the tank Q is fed by the pump N which receives it into a larger volume of water of a temperature above the melting point of sulfur which is being introduced into the 80 underground deposit.

The delivery of sawdust into the mine cavity is not a part of the ordinary working, but is effected at and during such times as it may appear to be called for. When introduced, a feed of about 100 pounds of sawdust per minute would represent a practical rate.

On September 19, 1906, patents respectively numbered 799,642 and 800,127 were granted on my said application of May 27, 1897, No. 638,357, and on a division of the same which was filed November 23, 1903, 90 and officially numbered 182,359.

I claim as my invention or discovery:

1. The improved process of fusion mining in porous deposits, which process is characterized not only by the introduction of fusion fluid into an underground porous 95 deposit of fusible material and by the removal of the melted material therefrom, but also by the introduction of comminuted material into said deposit in order thereby to restrict the freedom of movement of said fusion fluid in the deposit, substantially as described.

2. The improved process of fusion mining in porous deposits, which process is characterized not only by the introduction of fusion fluid into an underground porous deposit of fusible material and by the removal of the melted material therefrom, but also by the introduction 105 of comminuted material mixed with water into said deposit in order thereby to restrict the freedom of movement of said fusion fluid in the deposit, substantially as described.

3. In mining by fusion, the improvement consisting in introducing into an underground porous deposit comminuted material in admixture with water heated above the melting point of the material to be mined, and in removing the melted material, substantially as described.

4. In mining by fusion, the improvement consisting in melting the material in an underground porous deposit by hot water introduced without return into said deposit at a rate sufficiently above five hundred gallons a minute to prevent inroads into the melting space of naturally 110 present water from the surrounding rock, and in removing the melted material, substantially as described.

5. In mining by fusion, the improvement consisting in melting the material in an underground porous deposit by hot water introduced into said deposit, for such introduction supplying said hot water to the mine piping at a pressure above that corresponding with its temperature on leaving the heaters, causing the supply of so introduced water to flow away underground and so to hold back naturally present water, and removing the melted material, substantially as described.

6. In mining by fusion, the improvement consisting in effecting the melting by hot water introduced into an underground deposit which does not naturally admit of a pressure therein equal to that corresponding with the temperature of the hot water on leaving the heaters when added to the pressure of a water column the length of the mine piping, for such introduction supplying said hot water to the mine piping at a pressure above that corre-

- sponding with its temperature on leaving the heaters, causing the supply of so introduced water to flow away underground and so to hold back naturally present water, and removing the melted material, substantially as described.
7. In mining by fusion, the improvement consisting in introducing hot water into an underground porous deposit in order to melt the material therein, applying additional pressure to said water after heating and before its introduction into the deposit in order further to increase the rate of its delivery thereto, causing the supply of so introduced water to flow away underground and so to hold back naturally present water, and removing the melted material, substantially as described.
- 10 8. In mining by fusion, the improvement consisting in introducing hot water without return and comminuted material in admixture therewith into the underground deposit, and for such introduction supplying said hot water to the mine piping at a pressure above that corresponding with its temperature on leaving the heaters, and in removing the melted material, substantially as described.
- 15 9. The improved process of fusion mining in porous deposits, which process is characterized not only by the introduction of fusion fluid into an underground porous deposit of fusible material and by the removal of the melted material therefrom, but also by the introduction into said porous deposit of water without return and of comminuted material in admixture therewith, substantially as described.
- 20 10. In mining by fusion, the improvement consisting in introducing hot water without return and comminuted material in admixture therewith into an underground porous deposit, applying additional pressure to said water between the heaters and the mine piping, and removing the melted material, substantially as described.
- 25 11. In mining by fusion, the improvement consisting in heating water to a temperature above the melting point of the material to be mined by condensation of live steam therein under pressure, introducing the so heated water into an underground porous deposit, for such introduction supplying the so heated water to the mine piping at a pressure above that of said live steam, causing the supply of so introduced water to flow away underground and so to hold back naturally present water, and removing the melted material, substantially as described.
- 30 12. In mining by fusion, the improvement consisting in heating water to a temperature above the melting point of the material to be mined by condensation of live steam therein under pressure, introducing the so heated water into an underground porous deposit which does not naturally admit of a pressure therein equal to that of said steam when added to the pressure of a water column the length of the mine piping, for such introduction supplying the so heated water to the mine piping at a pressure above that of said live steam, causing the supply of so introduced water to flow away underground and so to hold back naturally present water, and removing the melted material, substantially as described.
- 35 13. In mining by fusion, the improvement consisting in melting the material in the underground deposit by hot water introduced partly through the pipe up which the melted material is raised in intervals between such raising and partly through separate hot water piping, causing both supplies of hot water to flow away underground and so to hold back naturally present water, and raising the melted material, the introduction of the hot water through the first mentioned pipe being stopped when the melted material is to be raised and the raising of said material being effected during such stoppage, substantially as described.
- 40 14. Apparatus for mining by fusion having a pipe up which the melted material is raised provided with a branch for delivering said material and a branch for receiving hot water for fusion, and separate hot water piping, said pipe and piping leading to an underground porous deposit and means being provided for closing the latter against return of water to the surface of the ground, substantially as described.
- 45 15. Apparatus for mining by fusion, having three pipes leading from hot water heaters to an underground deposit, one of which pipes is provided with a branch for delivery of melted material and also with means for shutting off the hot water connection during such delivery, the apparatus as a whole being arranged to confine the water from all the pipes to the deposit and so cause the supply from all of them to flow away underground, substantially as described.
- 50 16. Apparatus for mining by fusion, having means for introducing comminuted material into an underground deposit, and also having means for introducing fusion fluid into said deposit and for removing melted material therefrom, substantially as described.
- 55 17. Apparatus for mining by fusion, having means for introducing comminuted material in admixture with water into an underground deposit, and also having means for introducing fusion fluid into said deposit and for removing melted material therefrom, substantially as described.
- 60 18. Apparatus for mining by fusion, having means for introducing water at the fusing temperature into an underground deposit, and also means for allowing comminuted material to be mixed with said water, in combination with means for removing melted material from said deposit, substantially as described.
- 65 19. The combination of mine piping, means for supplying a mining fluid to the said mine piping, means for removing mined material, a mixing tank, a water supply for said tank, and connections between the said tank and the said mine piping, substantially as described.
- 70 20. The combination of mine piping, heaters, connections between the said heaters and the said mine piping, means for raising melted material through the said mine piping, a mixing tank provided with a stirrer, a water supply for said tank, and connections between the said tank and the said mine piping, substantially as described.
- 75 21. The combination of mine piping, means for raising melted material through said mine piping, a mixing tank, heaters, and connections between said mine piping and said mixing tank and heaters, substantially as described.
- 80 22. The combination with mine piping leading to an underground deposit of material to be mined, means for supplying fusion fluid to said piping, means for raising the melted material, and means whereby said deposit is closed against the return of the fusion fluid, of means for supplying comminuted material to said piping, substantially as described.
- 85 23. The combination of mine piping, means for raising melted material through said mine piping, a mixing tank, heaters, and pumps between said mine piping and said mixing tank and heaters, substantially as described.
- 90 24. The combination with mine piping leading to a porous deposit, means for raising melted material through said piping, and means whereby said deposit is closed against return of water to the surface of the ground, of heaters, and pumps between said heaters and said mine piping, substantially as described.
- 95 25. The combination with mine piping, means for raising melted material through said piping, and means for supplying hot water under pressure to said piping, of a mixing tank, and a pump receiving material from said tank and discharging it into said mine piping, substantially as described.
- 100 26. The combination of hot water heaters, mine piping, means for raising melted material through said mine piping, pumps between said heaters and said mine piping, and a mixing tank delivering material to a pump connected with said piping, substantially as described.
- 105 27. Apparatus for mining by fusion, in which water is heated by condensation of live steam in contact therewith, having pumps between such steam-condensing water heaters and the mine piping for forcing the so heated water through said piping into an underground deposit, and also having means for raising melted material from said deposit, and means whereby said deposit is closed against the return of the hot water to the surface of the ground, substantially as described.
- 110 28. Apparatus for mining by fusion having mine piping leading to an underground porous deposit, means for raising melted material from said deposit, means whereby said deposit is closed against the return of water to

the surface of the ground, and means which supply water heated above the melting point of the material to be mined to said mine piping at a rate sufficiently above five hundred gallons per minute to prevent inroads of 5 naturally present water from the surrounding rock, substantially as described.

29. Apparatus for mining by fusion, having hot water heaters and also having three pipes which lead from said heaters and open at different levels into an underground deposit of the material to be mined, means being provided for raising the melted material through that one of said pipes which opens into the deposit at the lowest level, and this last mentioned pipe being provided with a branch for delivery of the melted material raised through 10 the same and also with means for shutting off the water connection during such delivery, the apparatus as a whole being arranged to confine the water from all the pipes to the deposit and, so cause the supply from all of them to flow away underground, substantially as described.

30. Apparatus for mining by fluid, having means for introducing a mining fluid into a porous underground deposit of material to be mined, means for removing the mined material from said deposit, and means for introducing into the deposit comminuted material for choking 15 passages therein and thus restricting the freedom of movement of said mining fluid, substantially as described.

31. Apparatus for mining by fluid, having means for introducing a mining fluid into a porous underground deposit of material to be mined, means for removing the mined material from said deposit, and means for introducing 20 into the deposit at different levels comminuted material for choking passages therein and thus restricting the freedom of movement of said mining fluid, substantially as described.

32. Apparatus for mining by fluid, having means for introducing a mining fluid into a porous underground deposit of material to be mined, means for removing the mined mineral from said deposit by the pressure in said deposit, and means for introducing into the deposit comminuted material for choking passages therein and thus 25

restricting the freedom of movement of said mining fluid, substantially as described.

33. The process of mining by fluid, characterized not only by the introduction of mining fluid into a porous underground deposit of material to be mined and by the removal of the mined material, but also by the introduction into said deposit of comminuted material for choking 45 passages therein and thus restricting the freedom of movement of said mining fluid, substantially as described.

34. The process of mining by fluid, characterized not only by the introduction of mining fluid into a porous underground deposit of material to be mined and by the removal of the mined material, but also by the introduction into said deposit at different levels of comminuted material for choking passages therein and thus restricting 50 the freedom of movement of said mining fluid, substantially as described.

35. The process of mining by fluid, characterized not only by the introduction of mining fluid into a porous underground deposit of material to be mined and by the removal of the mined material, but also by the introduction into said deposit of comminuted material in the nature of sawdust for choking passages therein and thus restricting the freedom of movement of said mining fluid, 55 substantially as described.

36. The process of mining by fluid, characterized not only by the introduction of mining fluid into a porous underground deposit of material to be mined and by the removal of the mined material, but also by the introduction into said deposit of comminuted material of a specific 60 gravity not greater than that of water and in particles of about the size of sawdust for choking passages therein and thus restricting the freedom of movement of said mining fluid, substantially as described.

In testimony whereof I have signed my name to this specification in the presence of two subscribing witnesses.

HERMAN FRASCH.

Witnesses:

F. W. LOTHMAN,  
J. C. UPDEGROVE.